

## UNITED STATES PATENT OFFICE

2,046,061

## COATED METAL

Leo P. Curtin, Cranbury, and James M. Payne,  
Carteret, N. J., assignors to Curtin-Howe Cor-  
poration, New York, N. Y., a corporation of  
New York

No Drawing. Application January 10, 1935,  
Serial No. 1,258

17 Claims. (Cl. 148—6.5)

This invention relates to coated metals; and it comprises an article of steel or iron carrying a thin black surface layer containing vanadium in combination with oxalic acid, said layer being 5 hard, permanent, elastic enough to resist flexing to a marked degree and serving as a bonding agent between the metal and subsequently applied paint, cohering to both; and it further comprises a method of coating ferrous metal and 10 preparing it for painting wherein the cleaned or pickled ferrous metal is exposed to the action of a solution containing tetravalent vanadium and oxalic acid and is thereafter washed and dried; all as more fully hereinafter set forth and as 15 claimed.

In the metal finishing industry, it is now customary prior to painting to apply some type of a protecting coating to the clean metal; this preliminary coating serving as a basis for subsequent 20 painting, varnishing and enameling. For the most part, it is difficult to secure completely protective coatings with ordinary types of paints and varnishes applied directly to clean naked iron or steel. One type of preliminary coating often used 25 is that produced by the action of solutions of phosphoric acid or of acid phosphates, on iron. It contains ferrous phosphate and often other phosphates as well. A solution containing a manganous phosphate is sometimes used. When 30 such a phosphate coating is washed and dried, it serves as a good basis for varnish, paint and lacquer. These coating materials cohere or bond better to the phosphated surface than they do to the naked metal. Besides phosphoric acid, other 35 acids have been used as coating agents, the coatings consisting of metallic salts of the respective acids used.

A difficulty with most of these coatings of the prior art is that they do not resist flexing well; if 40 coated sheet metal is bent at a sharp angle, there is a tendency to open flaws and crevices. Coatings satisfactory in most other respects are apt to be deficient in this; the coated metal often will not stand the manipulation necessary in making 45 up various things; automobile bodies, for example. With a rupture in the coatings due to flexing, there is the possibility of what is called “creeping corrosion”; rust appears under the double coatings and spreads indefinitely. These 50 coatings, while customarily called “rustproof”, are actually more in the nature of rust retardants. In damp locations, with any fracture or abrasion of the coating which exposes bright metal, rusting of the whole surface ultimately occurs; the rust, however, perhaps devel-

oping at 10 per cent of the rate at which the bright metal alone would rust. The coating is therefore a rust retardant.

We have found that coatings satisfactory as a protective agent for iron and steel and as a bonding agent linking paint to iron or steel can be made with a solution containing vanadium oxalates; and that these coatings exhibit a further advantage in that they offer a considerable resistance to rupture by flexing. Sheet metal so 10 coated can be bent at a very sharp angle with no tendency for the coating to crumble, even at the inner edge of the bend. The coating improves the resistance of the sheet metal to sharp, heavy impact and is fairly resistant to high temperatures, even up to 300° C. In contradistinction to the usual types of coating, this may be described as rust-proofing; it is not merely rust 15 retarding.

By immersing clean pickled sheet metal in an 20 acidified solution of a vanadium oxalate, a dark, firmly cohering coating is formed and, after washing and drying, the underlying bright metal is wholly protected. The solution is made by dissolving vanadium tetroxid with the aid of oxalic 25 acid and the same chemicals are used in replenishment. A slight amount of oxalic acid in excess is employed but it is not necessary to have free acid present in greater amount than suffices to prevent hydrolysis of the vanadium oxalate. A 30 pH ranging from 1 to 3 serves well. The coating bath should be rather hot, somewhere between 50° C. and 99° C. The time of treatment varies from 4 to 5 minutes to several hours. With 4 or 5 minutes treatment, the bath ordinarily gives extremely thin black coatings; but the thickness is 35 sufficient for some purposes. A heavier type of coating is obtained with immersion for several hours. The color of the coating varies from a rich lustrous black to a dull black. It may be 40 made decorative, in event no after-painting is used. With a rich lustrous black in the coating and a layer of transparent varnish, decorative effects are obtained.

In making a typical coating bath in the present 45 invention, 166 parts of commercial vanadium tetroxid,  $V_2O_4$ , are dissolved in 10,000 parts of water with the aid of 260 parts of commercial oxalic acid. This bath contains the equivalent of 1.66 parts  $V_2O_4$  to 100 parts of water, but higher 50 and lower concentrations can be used. Good coatings can be produced with  $V_2O_4$  concentrations ranging from 0.3 to 4.0 per cent. A bath so prepared may be used indefinitely long with occasional replenishment of the contained vana- 55

dium and oxalic acid. The vanadyl oxalate may be used in the corresponding amount. Commercial vanadium pentoxid,  $V_2O_5$ , may be used in replenishing the bath; it being reduced by oxalic acid to the vanadyl form. Additions of oxalic acid should be in the amounts required to keep the bath clear. Should a sludge of insoluble ferrous oxalate or of insoluble reduced vanadium compounds form it can be cleared up by cautious 10 additions of strong commercial hydrogen peroxid solution in the right amount. Ferrous oxalate is converted into ferric oxalate. Weak solutions give an undesirable dilution and it is not advantageous to add enough peroxid to cause substantial oxidation in the bath itself. Bubbling air through the bath is sometimes expedient. An addition of  $V_2O_5$  can sometimes be utilized in producing the limited amount of oxidation wanted. The precise nature of the solute contained in the bath made as described ante is not known and it changes after use in coating ferrous metal. Reduction appears to take place; trivalent vanadium appearing. Ferrous oxalate is also present. Ferrous oxalate although insoluble 20 in water and in oxalic acid solutions, has a rather substantial solubility in a solution of vanadium oxalates. In the use of the bath with iron and steel, ferrous oxalate can be formed and go into solution. The presence of this ferrous oxalate in 25 solution is apparently desirable, up to concentrations of about, say, 0.5 per cent ferrous oxalate in the bath.

In forming the coating the iron metal is attacked and there is a production of ferrous oxalate, some of which becomes part of the coating. Some goes into the bath. In the coating, there are trivalent and tetravalent vanadium; there are derivatives of vanadium trioxid,  $V_2O_3$ . Vanadium forms a number of different oxids and 30 they combine among themselves, so that it is possible that intermediate oxids between the trivalent and tetravalent are present, these being in combination, probably, with the oxalyl radical, although "vanadites of vanadium" or of ferrous 35 iron may be present. In some instances the coating appears to contain a basic oxalate which may be a vanadyl oxalate corresponding to the formula  $V_2O_4 \cdot VO \cdot C_2O_4$ .

As stated, the bath always contains more or 40 less iron and this iron is useful in forming and contributing the coatings. It has been found that good coatings may be obtained with baths in which the amount of iron present is greater than that incident to the formation and solution 45 of ferrous oxalate. Small additions of ferrous oxalate are sometimes useful in bringing the bath to its steady state. Sometimes ferric oxalate is added. Good coatings can be made with a bath containing about equal proportions of vanadyl 50 oxalate and ferric oxalate; say about 1.5 per cent of each.

The composition of the coating layer in all cases is complex but whatever its composition, it has the described advantageous properties. Its 55 resistance to rusting is about four times as great as that of similar commercial "rustproofed" metal produced by prior processes. In comparative tests of the prior material and the present material, with plates or "panels" each carrying three 60 coats of lacquer, they were sharply scratched to expose bright metal and comparative observations made at weekly intervals showed about 4-fold resistance in the present material.

As stated ante, the coating is resistant to heat; 65 and, as a matter of fact, it is sometimes, for

special purposes, desirable to heat it. Heating may be up to a low red heat, or even by direct impingement of a flame. The color changes from black to dark blue. Undoubtedly, the oxalate radical breaks up. The bluish coating left after heating, however, has substantially the same desirable physical and chemical properties, as well as the rust resistance, as an unheated similar coating.

The coating bath in the present invention is 10 acid, having a pH between 1 and 3. Alkaline baths do not give the same results; a vanadium-containing, rust resisting coating on ferrous metal. In an acid solution, the vanadium is present as a cation and a coating is formed containing 15 vanadium without production of iron hydroxids; without rusting the metal.

As stated, the presence of iron compounds in the vanadium coating bath is often advantageous. Conversely, it is found that small additions of 20 vanadium compounds improve the action of other oxalate coating baths. Iron is commercially coated by treatment with a solution of ferric oxalate and a small addition of a vanadium compound to this bath improves the results; it gives a 25 better coating. The coating is darker and its rust resisting properties are considerably improved. Iron can be coated in a solution of oxalic acid alone although its action is rather slow and an addition of a small amount of vanadium 30 oxalate improves the results.

While we have particularly described the use of oxalic acid in making the bath, other organic acids may be used, but, as we at present think, with less advantage. Solutions made with citric 35 and tartaric acids give coatings which, made under the conditions described, are not as good as those made with oxalic acid. Phosphoric acid used as a substitute for oxalic acid in the directions given ante, produces a coating better than 40 is given by tartaric or citric acid under the same conditions. Good coatings can be made by these other acids, but their properties are somewhat different from those of the coating made with oxalic acid.

In all cases, the bath should be acid to the described extent, with a pH between 1 and 3. In preserving the desired acidity an addition of acid sodium oxalate is useful as a buffer salt.

What we claim is:—

1. As a new manufacture, a ferrous metal object having formed thereon a rustproofing coherent surface coating containing oxalates and vanadium.

2. The method of rustproofing ferrous metals 55 which comprises immersing such metal in a slightly acid solution containing vanadium as an oxalate.

3. The process of claim 2 wherein the slightly acid solution has a pH between 1 and 3. 60

4. The process of claim 2 wherein immersion is at a temperature between 50° and 99° C.

5. In the rustproofing of sheet metal, the process which comprises immersing a plurality of successive sheets in a replenished bath containing a 65 vanadium oxalate, replenishment being by additions of oxalic acid and  $V_2O_4$  and the tendency of both to deposit insoluble products being corrected by occasional oxidative treatments.

6. In the process of claim 5, as an oxidative 70 treatment, bubbling air through the solution.

7. In the process of claim 5, as an oxidative treatment, an occasional introduction of  $V_2O_5$ .

8. In the process of claim 5, introducing hydrogen peroxid as an oxidative treatment. 75

9. In rustproofing ferrous metal articles and providing a protective coating, the process which comprises immersing such an article in a replenished bath containing vanadium and iron as oxalates with enough excess oxalic acid to keep the solution clear, withdrawing, washing and drying.
10. In the process of claim 9, the method of replenishment which comprises occasional additions of  $V_2O_4$ , of oxalic acid in the amount necessary to keep the solution slightly acid and of an iron oxalate.
11. As a rustproofing method for ferrous metal, the process which comprises forming upon a ferrous metal article a coherent surface coating containing oxalates and vanadium and afterwards heating the article to break up the oxalyl radical.
12. The process of providing ferrous metal objects with a rustproofing coating which comprises immersing such an object in a slightly acid solution of a vanadium salt, the acidity having a pH value of 1 to 3.
13. As a new manufacture, a ferrous metal ob-
- ject having formed thereon a thin, black, hard, coherent surface coating of a vanadium compound, said coating being impervious and being resistant to rupture by flexing or impact.
14. The article of claim 13 wherein the coating containing vanadium has the characteristics of a baked vanadyl oxalate coating.
15. An article having a surface of ferrous metal having formed thereon a protective coherent oxalate coating containing a substantial amount of vanadium in addition to other metallic oxalates.
16. An article having a surface of ferrous metal having formed thereon a coherent protective coating containing a vanadium oxalate in addition to iron oxalate.
17. A process of providing ferrous metal objects with a rustproofing coating which comprises exposing such an object to the action of an acidulated solution containing a vanadyl salt of an acid of the group consisting of oxalic, citric, tartaric and phosphoric acid.

LEO P. CURTIN.  
JAMES M. PAYNE.